

## UNITED STATES PATENT OFFICE.

EDWARD VINCENT GARDNER, OF OXFORD STREET, AND PATRICK MOIR  
CRANE, OF MANCHESTER, ENGLAND.

## IMPROVEMENT IN COMPOSITIONS FOR COATING SHIPS, BOATS, &amp;c.

Specification forming part of Letters Patent No. 98,862, dated January 18, 1870; patented in England,  
March 13, 1869.

*To all whom it may concern:*

Be it known that we, EDWARD VINCENT GARDNER, of Oxford Street, in the county of Middlesex, England, and PATRICK MOIR CRANE, of Manchester, in the county of Lancaster, England, have invented a new or Improved Composition for Coating Ships, Boats, and other Surfaces, and for protecting and preventing the fouling thereof; and we do hereby declare that the following is a full and exact description thereof.

The nature of our invention consists in the employment of paraffine as the basis of a composition or compound to be used for coating ships, boats, and other surfaces to protect them and to prevent the fouling thereof.

The paraffine may be mixed with other ingredients, such as metallic filings or particles or metallic oxides. It may also be mixed with poisonous ingredients known to act injuriously to life, such as arsenic, sulphate of copper, compounds of mercury, and the like, according to the purposes to which the composition is to be applied. In some cases we use paraffine, in combination with creosote, dissolved in heavy oils. We also prepare a compound by vulcanizing paraffine with sulphur. In some cases, also, we combine tallow and rosin with the paraffine.

The invention, however, essentially consists in the employment of paraffine as the basis of a composition or compound to be employed for the purposes before described; and, in order that our invention may be fully understood, we will describe more fully how it may be carried into effect. The following proportions or parts we only give as approximate proportions, not confining ourselves thereto. For coating ships, vessels, boats, and some other purposes, we first take a composition composed of one or other of the following ingredients:

First coat: Either with white lead, white zinc, or red lead.

Second coat: Two parts white lead; two parts hard paraffine-wax; one part linseed-oil; one part rosin.

Third coat: One part oil, pressed from paraffine; one part rosin; one-half part hard paraffine-wax.

To either or all of these coats poisons or

poisonous materials may be added in any desired or convenient proportions. For this we prefer from one to two per cent. of white arsenic, cyanide of potassium, bichloride of mercury, strychnine, nux-vomica, extract of tobacco, or a mixture of these with other poisonous substances may be employed; or the third coat may be one-half part oil, pressed from paraffine, and one-half part hard paraffine-wax. This coat will do best for the portion of the ship's bottom not out of the water when she is light in cargo, with the necessary poison. These materials are melted in any convenient vessel, and put on hot, with brushes, in the usual way of coating vessels.

Coating for iron or metallic roofs, plates, sheets, girders, pipes, wires, and other purposes to which it may be applied, or structures composed of stone, metal, wood, bricks, tiles, or such like materials: Two parts hard paraffine-wax; one part rosin; one part white lead; or, three parts hard paraffine-wax; one part rosin; one part white lead.

We sometimes add to the above one-fifth to one-half part of kaoline, aluminous earths, silicious matters, and carbon or carbonaceous material. A compound produced by combining sulphur with paraffine, and called by us "vulcanized paraffine," is also well fitted for this purpose. These compositions may be put on when hot, with brushes; or, when convenient, the articles may be dipped in the composition.

What we claim as our invention, and desire to secure by Letters Patent, is—

The employment of paraffine as the basis of a composition or compound or of compositions or compounds, substantially in manner and for the purposes described.

EDWD. V. GARDNER, F. R. S., M. S. A.  
P. M. CRANE.

Witnesses to the signature of E. V. Gardner:

M. WYNN,  
24 Royal Exchange, London.

EDWD. GRIFFITH BREWER,  
89 Chancery Lane, London, W. C.

Witnesses to the signature of P. M. Crane:

JNO. B. PAYNE,  
Solicitor, Manchester.

C. DOUBOE,  
U. S. Consulate, Manchester.